

1

2,872,334

## ASPHALT CUTBACK, HARD FILM RUST PREVENTIVE

Michael J. Furey, Berkeley Heights, and Roy A. Westlund, Jr., Roselle, N. J., assignors to Esso Research and Engineering Company, a corporation of Delaware

No Drawing. Application February 2, 1956  
Serial No. 562,948

6 Claims. (Cl. 106—271)

This invention relates to improved rust preventive compositions and, more particularly, to improved compositions having utility as solvent-cutback, hard film rust preventives. More specifically, the invention relates to asphalt cutback rust preventive compositions which have been improved in low temperature flaking tendency by inclusion therein of a minor proportion of a microcrystalline wax.

Solvent-cutback, hard film rust preventives are known in the art. These are cold-applied compounds used for (1) the protection of metals exposed to a variety of outdoor weather conditions and (2) any general purpose preservation where a dry-to-touch film is desired. These materials generally contain an asphalt diluted with a petroleum solvent. The compounds are fluid in nature and may be applied to the metal surfaces to be protected by dipping, brushing or spraying. Upon evaporation of the solvent, a thin film, usually about 1 to 5 mils thick, remains on the metal parts to serve as protection against weathering, corrosive fumes, and the like. In addition, the protective coating should not flow from surfaces at high temperatures nor flake at low temperatures. When desired, the thin film is easily removed from the metal surfaces by the application of solvents such as petroleum solvents and the like.

Asphalts made by vacuum or steam reduction or by reduction followed by oxidation are desirable as base materials for use in certain solvent-cutback, hard film rust preventives because these asphalts have good storage stability and drying characteristics, give excellent protection, and are readily removed after exposure. They do, however, tend to be excessively brittle at low temperatures, and when cold give an undesirable degree of flaking or chipping from the metal surfaces being protected. This is particularly undesirable since the portion of the metal surface exposed is thus available for rusting and corrosion to an even greater degree than completely unprotected surfaces.

It has now been found and forms the object of this invention that this undesirable flaking tendency may be inhibited by the inclusion in these solvent-cutback, hard film rust preventive compositions of a minor amount of a microcrystalline wax. This discovery is indeed striking when it is considered that the microcrystalline wax per se is extremely brittle and flakes quite readily at the test temperatures.

The base material for the compositions of this invention comprises from 40 to 70% by weight of an asphalt and from 60 to 30% of a solvent therefor. The asphalt may be selected from the group of straight reduced asphalts or asphalts prepared by vacuum reduction to a solid flux with a penetration of less than 200 mm./10 followed by oxidation, with the latter being preferred. Especially preferred are asphalts which are vacuum reduced to a penetration of less than 70 mm./10 and then oxidized to a softening point between about 160° and 170° F. Asphalts prepared by oxidation of a liquid flux are not operable.

2

The solvent used in preparing the base material may be any of the well-known petroleum solvents having flash points between about 100° and about 150° F. and mid-boiling points ranging from about 300° to about 350° F. with a final boiling point below about 410° F. If it is desired, blends of various solvents having FBP below about 410° F. may be used as the diluent for the asphaltic material.

In accordance with the concept of the instant invention, hard film, solvent-cutback rust preventive compositions were formulated from the following components.

### THE ASPHALT COMPONENT

Several different asphalts were used in preparing blends in accordance with this invention.

#### 15 Asphalt A

This asphalt is a reduced asphalt made by the vacuum reduction of a Columbian crude. This material, a straight reduced asphalt, had a softening point of about 146° F.

#### 20 Asphalt B

This asphalt was prepared by vacuum reduction of a Venezuelan (Lagunillas) crude to a liquid flux having a flash point of about 500 to 505° F. This flux was then oxidized by air blowing at about 425° F. to a softening point of 160° to 180° F.

#### 25 Asphalt C

This asphalt was prepared by vacuum reduction of a Venezuelan (Lagunillas) crude to a 500/505° F. flash point liquid flux followed by oxidation by air blowing at about 425° F. to a softening point of 220° to 235° F.

#### 30 Asphalt D

35 A fourth asphalt was prepared by vacuum reducing a Venezuelan (Lagunillas) crude to obtain a solid flux having a 20 to 30 penetration at 77° F. This material was then air blown at about 425° F. to a softening point of 160 to 170° F.

#### 40 Asphalt E

45 A fifth asphalt was prepared by vacuum reducing a Venezuelan (Lagunillas) crude to a solid flux with a 41 to 60 penetration followed by air blowing at about 425° F. to a softening point of 160° to 170° F.

### SOLVENTS

In the composition two different solvents were used. Solvent A was a highly refined virgin cut petroleum solvent from a low sulfur paraffinic crude having the following inspections:

|                           |      |
|---------------------------|------|
| Flash point (tag), ° F.   | 105  |
| Kauri-butanol number      | 38.0 |
| Aniline point, ° F.       | 129  |
| Percent off at 340° F.    | 50   |
| Percent off at 375° F.    | 90   |
| Final boiling point, ° F. | 405  |

50 Solvent B was an aromatic petroleum solvent having more than 95% aromatics and having the following inspections:

|                             |     |
|-----------------------------|-----|
| Flash point, ° F.           | 107 |
| Initial boiling point, ° F. | 300 |
| Percent off at 330° F.      | 50  |
| Percent off at 350° F.      | 90  |
| Final boiling point, ° F.   | 370 |

### MICROCRYSTALLINE WAX

70 The waxes used were microcrystalline waxes having a melting point above 170° F. These waxes were prepared by conventional solvent dewaxing of petrolatums or by

the solvent dewaxing of the residuum settling out of crude storage tanks. Inspections on these waxes are as follows:

| <i>Wax A</i>                   |          |
|--------------------------------|----------|
| Color (N. P. A.)               | 3½       |
| Flash point                    | ° F 560  |
| Fire point                     | ° F 590  |
| Viscosity @ 210° F             | SSU 87   |
| Acid No. (ASTM D-974)          | 0        |
| Saponification No. (ASTM D-94) | 0        |
| Penetration (ASTM D-5)         | mm./10 4 |
| M. P. (ASTM D-127)             | ° F 192  |

| <i>Wax B</i>                   |           |
|--------------------------------|-----------|
| Color (N. P. A.)               | -----     |
| Flash point                    | ° F. 550  |
| Fire Point                     | ° F. 610  |
| Viscosity @ 210° F.            | SSU 113   |
| Acid No. (ASTM D-974)          | 0         |
| Saponification No. (ASTM D-94) | 0         |
| Penetration (ASTM D-5)         | mm./10. 3 |
| M. P. (ASTM D-127)             | ° F. 193  |
| Specific gravity @ 60° F.      | 0.9433    |

As was stated above, the hard film solvent cutback rust preventive compositions of this invention are prepared by incorporating into a base material a minor amount of a microcrystalline wax at temperatures above the melting point of the wax. Operable and preferred amounts of the components of the blends are set out below:

| Component     | Operable Range (wt. percent) | Preferred Range (wt. percent) |
|---------------|------------------------------|-------------------------------|
| Asphalt.....  | 40.0-70.0                    | 53.0-63.                      |
| Solvent.....  | 29.0-59.0                    | 34.0-44.                      |
| Microwax..... | 1.0-8.0                      | 3.0-5.0                       |

In accordance with the concept of the instant invention several blends were prepared. These blends were submitted to the following standard tests for hard film rust preventive compositions.

(1) *Film thickness*.—This test is conducted as follows: A steel test panel, 2" x 4" x  $\frac{1}{8}$ ", is finished by polishing with 240 grit aluminum oxide abrasive with cloth or paper backing to a surface finish of 10-20 micro inches (root means square). The panel is then wiped clean and rinsed in boiling naphtha, then in boiling methanol and allowed to cool in a desicator to  $77 \pm 2^\circ$  F. The panel is weighed and then immersed for one minute in the test compound maintained at  $77 \pm 2^\circ$  F. The panel is withdrawn at the rate of 4 inches per minute and hung to dry in the laboratory. After 24 hours drying the panel

is reweighed and the film thickness calculated by the specific gravity weight method.

(2) *Drying time.*—This test is conducted as follows:

A test panel is coated as in the film thickness test and allowed to hang in the laboratory for 4 hours. At the end of this time the panel is handled, using normal finger pressures. Any transfer of the compound or injury to the film from handling fails this test.

(3) *Salt spray test*.—This test is conducted as follows:

Steel test panels are prepared and coated as in the film thickness test and dried for 24 hours in the laboratory. The panels are then placed in a salt spray cabinet conforming to Method 4001.1 of Federal Specification VV-L-791E and exposed for 14 days. At the end of this time the panels are removed, cleaned with solvent, and examined for rust. Any panel showing no more than 3 corrosion spots, no one of which is larger than 1 mm. in diameter, passes this test. Corrosion within  $\frac{1}{4}$ " of the panel edges is not considered in this evaluation.

(4) *Weather-O-Meter test*.—This test is conducted as follows:

Steel test panels are coated and dried as for the salt spray test. They are then exposed to the test described in Method 615.1 of Specification TT-P-141 for 1200 hours. At the conclusion of the test the coating is removed and the panel examined for signs of rust. Corrosion within  $\frac{1}{4}$ " of the panel edge shall be disregarded. Any panel showing no more than 3 corrosion spots, no one of which is larger than 1 mm. in diameter, passes the test.

(5) *Low temperature adhesion test.*—This test is conducted as follows:

Panels are coated as in the film thickness test and dried for 24 hours. The panel is then cooled to 0° F. for one hour and 4 parallel scratches approximately  $\frac{1}{8}$ " apart and one inch long made on the film with the scratch tool. Four similar scratches shall be made perpendicular to the first four. Chipping of the coating extending more than  $\frac{1}{2}$ " from either side of the scratch marks shall be considered a failure. The scratch tool consists of four razor blades held parallel and  $\frac{1}{8}$ " apart by a metal holder.

(6) *Thirty-day storage test*.—This test is conducted as follows:

Steel panels are coated and film thickness measured as in the first test above. The compound is then stored in the laboratory at  $77 \pm 5^{\circ}$  F. for 30 days. At the end of this time the compound is mixed by rolling a tightly sealed 0.9 full can at approximately 50 R. P. M. for 5 minutes. A second set of panels are then coated as before and the film thickness measured. Any increase in film thickness exceeding 15% fails the storage test.

In Table I below, there is set out the composition of these blends and the test results.

TABLE I.—HARD FILM SOLVENT OUTBACK RUST PREVENTIVES

A careful examination of the data set out in Table I shows the outstanding advantages of the blends prepared in accordance with the inventive concept. It is to be seen that the inclusion of from 3 to 5% of a microcrystalline wax is essential to enable the rust preventive to pass all the tests set out above. In addition, the asphalt must be either a straight reduced asphalt (A) or one prepared by oxidation of a solid flux prepared by reduction (D or E). Addition of the microcrystalline wax to asphalts prepared by oxidation of liquid fluxes (B or C) gives unsatisfactory products.

One outstanding composition prepared in accordance with the inventive concept has the following components.

55.0 wt. percent reduced and oxidized asphalt (160/170° F. S. P.)

36% solvent A

5% solvent B

4% wax A

This composition was tested according to Military Specification MIL-C-16173-A, grade I for solvent cutback rust preventives, hard film. Results of these tests are set out in Table II below:

TABLE II.—SPECIFICATION MIL-C-16173-A TESTS

| Test                                | Blend No. 8 |
|-------------------------------------|-------------|
| Flash Point (100° F. Min.)          | Pass        |
| Removability after Exposure         | Pass        |
| Film Thickness (4.0 Mil. Max.)      | 3.0         |
| Salt Spray, 14 Days                 | Pass        |
| Accelerated Weathering, 1,200 Hours | Pass        |
| Recovery From Low Temperature       | Pass        |
| Sprayability @ 40° F.               | Pass        |
| Low Temperature Adhesion (0° F.)    | Pass        |
| Drying Time, 4 Hours                | Pass        |
| Solvent, (410° F. Max. End Point)   | Pass        |
| Corrosion                           | Pass        |

ALLOWABLE LIMITS

| Immersion: |                           |  |       |
|------------|---------------------------|--|-------|
| Brass      | ±1.0 mg./cm. <sup>2</sup> |  | -0.03 |
| Cadmium    | ±5.0 mg./cm. <sup>2</sup> |  | 0.00  |
| Zinc       | ±7.5 mg./cm. <sup>2</sup> |  | +0.01 |
| Magnesium  | ±0.5 mg./cm. <sup>2</sup> |  | -0.01 |
| Aluminum   | ±0.2 mg./cm. <sup>2</sup> |  | -0.02 |
| Steel      | ±0.2 mg./cm. <sup>2</sup> |  | -0.02 |
| Coating:   |                           |  |       |
| Brass      | ±1.0 mg./cm. <sup>2</sup> |  | 0.00  |
| Cadmium    | ±5.0 mg./cm. <sup>2</sup> |  | +0.11 |
| Zinc       | ±7.5 mg./cm. <sup>2</sup> |  | 0.00  |
| Magnesium  | ±0.5 mg./cm. <sup>2</sup> |  | +0.02 |
| Aluminum   | ±0.2 mg./cm. <sup>2</sup> |  | 0.00  |
| Steel      | ±0.2 mg./cm. <sup>2</sup> |  | +0.02 |

It is to be seen that this composition was quite satisfactory in all portions of this test.

To summarize briefly, the instant invention relates to hard film solvent cutback rust preventive compositions. Compositions of the invention comprise from 40.0 to 70.0 wt. percent, preferably from 53% to 63% of a reduced or a reduced and oxidized asphalt having a softening point between 140° and 250° F., preferably between

160° to 170° F., from about 29.0 to about 59.0 wt. percent of a solvent having a final boiling point of within the range of from 350 to 450° F., preferably from 34.0 to 44.0 wt. percent of a solvent having a final boiling point between about 360° and 410° F., and about 1.0 to 8.0 wt. percent, preferably about 3.0 to 5.0 wt. percent, of a microcrystalline wax having a melting point above about 175° F. and a penetration of less than 10 mm./10.

What is claimed is:

- 10 1. A solvent cutback hard film rust preventive composition which consists essentially of a blend of from about 53% to about 63% of an asphalt selected from the class consisting of straight reduced asphalts having a softening point of from about 140° F. to about 250° F. and asphalts prepared by reduction to a solid flux having a penetration of less than 200 mm./10 at 77° F. followed by oxidation to a softening point of from about 140° F. to about 250° F., about 34% to about 44% of a petroleum solvent having a final boiling point within the range of from 350° to 450° F., and about 3% to about 5% of a microcrystalline wax having a melting point above 175° F. and a penetration at 77° F. less than 10 mm./10, said percentages being by weight based on the weight of the total composition.
- 15 2. A rust preventive composition according to claim 1 wherein said asphalt is a reduced and oxidized asphalt.
- 20 3. A rust preventive composition according to claim 1 wherein said solvent has a final boiling point of between 360° and 410° F.
- 25 4. A rust preventive composition according to claim 1 wherein said asphalt is a reduced asphalt.
- 30 5. A solvent cutback hard film rust preventive composition which consists essentially of a blend of about 53% to about 63% of an asphalt prepared by reduction to a solid flux having a penetration at 77° F. of less than 70 mm./10 followed by oxidation to a softening point of about 160° to 170° F., about 34% to about 44% by weight of a petroleum solvent having a final boiling point within the range of about 360° to about 410° F., and about 3.0 to 5.0 wt. percent of a microcrystalline wax having a melting point above 175° F. and a penetration at 77° F. less than 10 mm./10.
- 35 6. A solvent cutback hard film rust preventive composition which consists essentially of a blend of about 55.0 wt. percent of an asphalt prepared by reduction to a solid flux having a penetration at 77° F. of less than 70 mm./10 followed by oxidation to a softening point of about 160° to about 170° F., about 41.0 wt. percent of a petroleum solvent having a final boiling point of about 405° F., and about 4.0 wt. percent of a microcrystalline wax having a melting point above 175° F. and a penetration at 77° F. less than 10 mm./10.

References Cited in the file of this patent

UNITED STATES PATENTS

- 55 2,573,878 Schiermeier et al. Nov. 6, 1951  
2,641,551 Smith et al. June 9, 1953